

Patented May 21, 1929.

1,714,038

# UNITED STATES PATENT OFFICE.

ALPHONSUS F. MURPHY, OF ZANESVILLE, AND WILLIAM JONES, OF MIDDLETOWN, OHIO, ASSIGNEES TO THE AMERICAN ROLLING MILL COMPANY, OF MIDDLETOWN, OHIO, A CORPORATION OF OHIO.

## PROCESS OF TREATING SILICON STEEL.

No Drawing.

Application filed April 15, 1927. Serial No. 184,172.

Our invention relates to processes for the formation of smooth finish, scale free electrical sheets, formed of high silicon alloy steel, which sheets have been both pickled and annealed.

Otto Graef in his Patent No. 1,173,951, dated February 29, 1916, refers to the method of preparing silicon steel sheets by first pickling them, and then annealing them, in order to produce a scale free product, but in his patent states that by first annealing and then pickling, he obtains better electrical properties.

Our investigations with both processes have resulted in development of a process, whereby a certain type of pickling of silicon steel sheets, followed by a cold rolling to impart surface conditions, and followed by the usual annealing treatment to impart electrical properties, will result in a sheet of smooth finish, with the electrical properties as high or higher than can be obtained with the process of Graef, and with a space factor which is close to 100 per cent.

Among other things, the Graef patent fails to state the nature of the pickling step of his process, or of old processes which he believes himself to have improved, and we find that in order to remove the heavy mill scale resulting from the rolling of the sheets, it is necessary to provide a pickling solution and proper temperatures therefor, which will lift the scale fully, without pitting the sheets.

We will describe in detail the preferred mode of practicing our process, and will set forth the novelty inherent therein in the claims that follow.

In preparing the sheets for our treatment, they are hot rolled in packs, and the packs opened, and the sheets straightened out, as by giving them a pass between rolls, the object being to provide a sheet which is flat, so as to be readily handled in the treatment to follow. We thus pass the stripped sheets from the pack through a cold roll mill, either in the presence of water or dry, and if we can avoid this flattening process, we prefer to do so, since the finish to the sheet is imparted by a cold roll treatment after pickling, and a preliminary cold rolling tends to make the mill scale more adherent. Any mode of flattening the sheets following stripping the packs, will serve our purpose.

The sheets from the flattening step, if this

is required, are then passed to the pickling bath which is made up of a solution of sulphuric acid as usual in pickling, to which may be added with advantage, some suitable controlling solution such as are on the market. "Incontrol" is the trade name of a suitable product for this purpose. The object of controlling the pickling action is to lift the scale without rupturing the sheet. Substances such as Incontrol contain gelatinous materials, blood and preservatives and retard hydrogen development by shielding the cathodes during electrolytic action.

When the sheet has been pickled so as to be free of scale, it is thoroughly washed, with the final washing being given by a basic solution, such as a solution of water and air slaked lime, to neutralize the acid. Some other neutralizing solution can be employed instead of the lime, and following the neutralization, the sheets are thoroughly boshed and scrubbed mechanically, after which a mechanical separator is imposed on the sheets, such as by spraying them with air slaked lime solutions which dries to form a coating that keeps the sheets from adhering to each other during annealing.

The sheets, free from pit holes, and free from any acid, and coated with a mechanical separator, are piled in annealing boxes and given an annealing to produce the required magnetic properties. The sheets are then cold rolled, by being given one or more passes, preferably in the presence of water.

If this cold rolling be omitted, the results will be satisfactory, but not so valuable in producing a clean, smooth surface, as if the cold rolling is followed. Thus, the sheets without any surface imparting cold rolling, will be better than sheets which have not been pickled before annealing, but will not be so excellent as those which we produce by adding the cold rolling step.

The sheets are then again piled in annealing boxes and annealed at the temperatures and time periods known to be necessary for retaining and producing high electrical properties for the grade of material in question, after it has been worked.

When the second annealing cycle has been completed, the finished sheets will be smooth, and of a beautiful, clear finish, without traces of scale, and with a space factor which is practically one hundred per cent. By space

factor is meant the proportion of solid metal to solid metal, plus surface irregularities and scale or oxide, in a pile made up of a number of layers of the sheets.

5 Having thus described our invention, what we claim as new and desire to secure by Letters Patent, is:—

1. A process for preparing silicon steel sheets for electrical purposes, which consists in passing the manufactured sheets through a pickling treatment, then washing and cleaning away the acid, then annealing the sheets, then cold rolling the sheets, and finally re-annealing the sheets.

15 2. A process for preparing silicon steel sheets for electrical purposes, which consists in passing the manufactured sheets through a pickling treatment formed of sulphuric acid and a controlling solution to prevent pitting, cleaning the acid from the

sheet, neutralizing the sheets by treating with a basic solution, imposing a mechanical separator on the sheets, and annealing the product to produce electrical qualities, and finally giving a smooth surface to the sheets as by cold rolling, followed by a second annealing.

25 3. A process for preparing silicon steel sheets for electrical purposes, which consists in passing the manufactured sheet through a pickling treatment to remove the scale resulting in manufacture of the sheet, then cleaning the sheet, then neutralizing the sheets and imposing a mechanical separator thereon, and finally annealing the sheets to give electrical properties in two separate cycles, 30 intermediate of which cycles a surface smoothing treatment is imparted to the sheets.

35 ALPHONSUS F. MURPHY.  
WILLIAM JONES.